

## UNITED STATES PATENT OFFICE.

FREDERICK M. BECKET, OF NEW YORK, N. Y., ASSIGNOR TO ELECTRO METALLURGICAL CO., A CORPORATION OF WEST VIRGINIA.

## SEAMLESS HOLLOW ARTICLE AND PROCESS OF MAKING SAME.

No Drawing.

Application filed October 15, 1925. Serial No. 62,658.

This invention relates primarily to the manufacture of seamless tubing or other hollow articles from alloys of the general type known as "chrome-irons", which are characterized by their great resistance to corrosion particularly by their resistance to oxidation at high temperatures.

It has heretofore been possible to make tubing of chrome-iron alloys by the process of cutting rolled sheets into strips, forming these into cylinders and subsequently welding them by means of gas or electricity to form a tube. This method is entirely practicable and results in a product which is satisfactory for many purposes; however, for many purposes, especially where a thick walled tube is required there are certain disadvantages inherent in the welded tubes. Among these are difficulties in welding heavy walls, danger of porous spots in the welds and rather large unit cost. A seamless tube possesses the further advantages of being more substantial or strong mechanically and not liable to open up as a result of repeated expansion strains due to alternate heating and cooling.

Under these conditions it is natural that many efforts should have been made in the past to make seamless tubing from various compositions of iron-chromium alloys, using the methods which have proven successful in the manufacture of seamless tubing from steel. Many such attempts have been made, but in no case, so far as I am aware, have they been successful; and it is the present general opinion among metallurgists that there is little prospect of an industrial solution of the problem.

It is well-known to those skilled in the manufacture of seamless tubing from steel by the Mannesmann or similar process that the piercing of the billet not only forms the initial hole but tears the walls of it to a greater or less extent; but that in the subsequent hot working, the rolling and pressing movements autogenously weld the tears to produce and in this way effectively heal these ruptures. Knowing that chrome-irons once torn will not re-weld even under the most favorable conditions of temperature and pressure which have yet been brought to bear upon them, it has naturally been concluded by those skilled in this art that the manufacture of seamless tubing from chrome-iron, and especially from iron-chro-

mium alloys relatively high in chromium, containing, say, upward of about 10% of chromium would be impossible by any methods now available. The extreme hardness and toughness of chrome-iron alloys at high temperatures, such as are normally used in similar operations upon steel, has strongly confirmed this opinion.

Nevertheless, in determining the tensile strength of a variety of chrome-irons, including those of chromium contents both above and below 20% of chmorium, I have observed a great and unexpected ductility in these alloys within the range of temperature lying approximately between 1000° and 1175° C.; and my experimentation has shown that many of the most useful chrome-irons moderately low in carbon can be successfully pierced from billets and rolled to seamless tubes through the employment of appropriate modifications of standard processes and by the use of existing machinery and pre-heating equipment.

Taking advantage of the above observation I have successfully pierced billets of various chrome-irons and have rolled the pierced billets to seamless tubes of standard dimensions and merchantable lengths. For example, I have found it commercially practicable to pierce and roll to excellent seamless tubing iron-chromium alloys of the following approximate compositions, the balance in each case being chiefly iron:

|     |       |                 |
|-----|-------|-----------------|
| Cr. | 26.89 | 24.37           |
| C.  | 0.25  | 0.18 00         |
| Si. | 0.44  | 0.37            |
| Mn. | 0.53  | 0.96            |
| P.  | 0.018 | Not determined. |
| S.  | 0.02  | Do              |
| Ni. | 0.542 | Do 95           |

My invention is not restricted however to an iron-chromium alloy of the above approximate composition, since the composition may vary rather widely without becoming unsuitable for my purpose. The above mentioned alloys are however typical of those which are highly resistant to oxidation even at high temperatures, and are for this reason especially valuable in the form of seamless tubing: but my invention contemplates broadly, the application for this purpose of all such iron-chromium alloys as resemble those whose composition is given above in the possession of sufficient ductility to allow of their being converted into seam-

less tubing by proper modification of known methods, such for instance as the so-called shell-piercing method. Nickel and other alloying elements may be present in any pro-

5 portion which will not interfere with the essential properties of the metal for my specific purposes.

For the greatest facility of working, the 10 carbon content of the alloy should be as low as practicable. For example a chrome-iron of carbon content 0.25% or lower has been found to pierce and roll much more easily than a similar alloy having a carbon content materially higher than 0.25%.

15 Maximum limits of chromium and carbon, or of alloying elements, cannot however be stated, as these will of course depend upon the strength of piercing points, and the strength and power capacity of the piercing machinery available for the work. It is of course recognized that there must exist an upper limit of carbon content at which an alloy of any particular chromium content will lose that measure of ductility 20 which is essential to the success of the operation.

Seamless steel tubing is made by piercing billets of low carbon steel by the Mannesmann, Steifel or similar process and subsequently rolling to the desired calibre and thickness of wall. The steel billet is pierced 30 preferably within the range of 1250° to 1350° C., and even higher temperatures are hazarded in order to secure greater softness and a consequent increase in the speed of 35 piercing. The upper limit of temperature is indicated by the appearance of incipient red-shortness. In heating steel billets preparatory to piercing, and particularly 40 through the higher temperatures of the pre-heating ranges, the furnace atmosphere must be maintained in a reducing condition in order to avoid superficial oxidation of the steel, a condition unfavorable to the quality 45 and appearance of the finished tube.

In contradistinction to the above conditions which govern the making of steel tubing, the temperatures which I have found best adapted for the piercing of billets of 50 the various chrome-irons,—and especially those having chromium contents of 20% and upward,—lie below about 1175° C. and in most cases at least within the range 1000°–1175° C.

55 At temperatures substantially below 1000° C. piercing of the commercial varieties of chrome-iron becomes difficult; and above about 1200° C. they develop red-shortness.

60 In heating the billets preparatory to piercing, the furnace need not present a reducing atmosphere, as in the case of steel billets, since the resistance of the commercial varieties of chrome-iron to oxidation at high temperatures establishes a wide tolerance 65 of oxidizing conditions. On the other hand

in the upper part of the pre-heating range, and notably above 1000° C., prolonged exposure to a highly reducing furnace atmosphere will embrittle these alloys.

In heating billets of the chrome-irons the 70 rate of rise in temperature, especially up to about 600° C., is preferably quite slow as compared with that permissible and employed in heating billets of steel, in order to avoid any tendency to cracking the 75 chrome-iron. After reaching red-heat, the subsequent rise in temperature can well proceed as rapidly as is now usual in heating steel for billet-piercing. But before piercing I have found it desirable to hold the 80 billet of chrome-iron at the piercing temperature until all parts of it have reached approximately the same temperature, in order that the deformation of the alloy and the resulting strains arising from the piercing 85 operation may not tend to crack the billet.

As an illustrative example of the preheating of chrome-iron for the manufacture of 90 seamless tubing, the cold billets are placed in a reheating furnace of the usual type, in which they are slowly preheated to about 600° C. over a period varying between 1½ and 3 hours. Thereafter the billets are raised as rapidly as desired to the temperature selected for piercing—usually between 1050° and 1150° C. This is commonly accomplished in about 3 hours, and the billets are usually held at the piercing temperature for an additional hour or more in order 100 to equalize the temperatures of all the billets of the batch, as well as to secure a uniform temperature throughout the material of each billet. Each billet is then pierced, and 105 rolled into seamless tubing of the desired dimensions.

For the manufacture of seamless tubing by hot piercing and rolling, chrome-iron alloys should be produced, poured, cast and 110 rolled under conditions which will provide billets free of slag, oxides and other non-metallic inclusions. They should also contain the minimum of dissolved oxides or other impurities either dissolved or chemically combined, which can contribute to 115 embrittling the billet at the temperatures used for piercing or in the subsequent rolling. I have found that inclusions as well as impurities dissolved or otherwise contained in chrome-irons may render them unsuitable or even useless as material for hot-piercing and subsequent rolling to seamless tubes.

I have found that seamless tubes of 120 chrome-iron can also be made by hot-piercing a cylindrical billet to form a cup, cropping the cup to an open cylinder, and rolling the latter into tubing of the required dimensions. I have also made hot-drawn or 125 hot-pressed pots or containers of chrome- 130

iron by means of standard machinery commonly used for the drawing or pressing of the similar vessels from steel, by an application of the methods above described in connection with the operation of making seamless tubing. Hence I employ the term seamless tubing herein in its broad significance, as including seamless hollow articles of various kinds.

10 The range of usefulness and the variety of appropriate applications of seamless tubing made of chrome-iron are obvious. Tubing produced from these alloys may prove almost indispensable as an element of construction in furnaces, recuperators, superheaters, autoclaves and stills, and in many other forms of equipment and apparatus which encounter high temperatures as well as erosive and corrosive agencies. For all 15 such applications chrome-iron tubing offers the ease of fabrication and high thermal conductivity common to most metals and alloys, and in addition presents a combination of strength and resistance to oxidation 20 at high temperatures, as well as resistance to many forms of corrosion, which are not simultaneously found in any other metal or alloy.

I claim:

30 1. Process of making a seamless hollow article by hot piercing followed by working such as rolling or drawing, comprising piercing an iron-chromium alloy containing at least about 10% of chromium at a tem-

perature lying approximately between 35 1000° and 1175° C.

2. Process of making a seamless hollow article by hot piercing followed by working such as rolling or drawing, comprising 40 piercing an iron-chromium alloy containing at least 20% chromium, at a temperature lying approximately between 1000° and 1175° C.

3. Process of making a seamless hollow article by hot piercing followed by working 45 such as rolling or drawing, comprising piercing an iron-chromium alloy containing approximately 25% chromium, at a temperature lying approximately between 1000° and 1175° C.

4. A hollow article of the character described having seamless walls of an iron-chromium alloy containing at least 10% chromium produced by a hot-piercing operation.

5. A hollow article of the character described having seamless walls of an iron-chromium alloy containing at least 20% chromium produced by a hot-piercing operation.

6. A hollow article of the character described having seamless walls of an iron-chromium alloy containing approximately 25% chromium produced by a hot-piercing operation.

In testimony whereof, I affix my signature.

FREDERICK M. BECKET.